



US011697908B2

(12) **United States Patent**  
**Giuste et al.**

(10) **Patent No.:** **US 11,697,908 B2**  
(b4) **Date of Patent:** **Jul. 11, 2023**

(54) **SMOOTH AND LOW DENSITY PAPERBOARD STRUCTURES AND METHODS FOR MANUFACTURING THE SAME**

(71) Applicant: **WestRock MWV, LLC**, Atlanta, GA (US)

(72) Inventors: **Sergio A. Giuste**, Midlothian, VA (US); **Steven Parker**, Raleigh, NC (US); **Terrell J. Green**, Raleigh, NC (US)

(73) Assignee: **WestRock MWV, LLC**, Atlanta, GA (US)

(\*) Notice: Subject to any disclaimer, the term of this patent is extended or adjusted under 35 U.S.C. 154(b) by 0 days.

(21) Appl. No.: **17/683,454**

(22) Filed: **Mar. 1, 2022**

(65) **Prior Publication Data**

US 2022/0267961 A1 Aug. 25, 2022

**Related U.S. Application Data**

(62) Division of application No. 16/869,156, filed on May 7, 2020, now Pat. No. 11,293,142.

(60) Provisional application No. 62/846,278, filed on May 10, 2019.

(51) **Int. Cl.**

**D21H 19/58** (2006.01)  
**D21G 1/02** (2006.01)  
**D21H 19/38** (2006.01)  
**D21H 19/40** (2006.01)  
**D21H 19/54** (2006.01)  
**D21H 19/82** (2006.01)  
**D21H 23/30** (2006.01)

(52) **U.S. Cl.**

CPC ..... **D21H 19/58** (2013.01); **D21G 1/0246** (2013.01); **D21G 1/0253** (2013.01); **D21H 19/385** (2013.01); **D21H 19/40** (2013.01); **D21H 19/54** (2013.01); **D21H 19/822** (2013.01); **D21H 23/30** (2013.01)

(58) **Field of Classification Search**

CPC ..... D21H 19/40; D21H 19/58; D21H 19/822; D21H 19/385; D21H 19/54; D21H 19/82; D21H 25/14; D21H 23/30; D21G 1/0246; D21G 1/0253

USPC ..... 162/136  
See application file for complete search history.

(56) **References Cited**

**U.S. PATENT DOCUMENTS**

|             |         |                 |
|-------------|---------|-----------------|
| 4,749,445 A | 6/1988  | Vreeland        |
| 4,823,688 A | 4/1989  | Wedel et al.    |
| 4,888,983 A | 12/1989 | Dunfield et al. |
| 5,245,920 A | 9/1993  | Hess            |
| 5,298,335 A | 3/1994  | Reed et al.     |
| 5,320,672 A | 6/1994  | Whalen-Shaw     |

|                 |         |                    |
|-----------------|---------|--------------------|
| 5,378,497 A     | 1/1995  | Johnson et al.     |
| 5,631,080 A     | 5/1997  | Fugitt             |
| 5,690,527 A     | 11/1997 | Rutledge et al.    |
| 6,200,424 B1    | 3/2001  | Saari et al.       |
| 6,274,001 B1    | 8/2001  | Mohan              |
| 6,582,553 B2    | 6/2003  | Jewell et al.      |
| 6,698,342 B1    | 3/2004  | Heikkinen et al.   |
| 6,777,075 B2    | 8/2004  | Concannon et al.   |
| 6,802,938 B2    | 10/2004 | Mohan et al.       |
| 6,866,906 B2    | 3/2005  | Williams et al.    |
| 7,208,039 B2    | 4/2007  | Jones et al.       |
| 7,306,668 B2    | 12/2007 | Pring et al.       |
| 7,425,246 B2    | 9/2008  | Urscheler          |
| 7,504,002 B2    | 3/2009  | Brelsford et al.   |
| 7,749,583 B2    | 7/2010  | Fugitt et al.      |
| 8,142,887 B2    | 3/2012  | Fugitt et al.      |
| 9,567,709 B2    | 2/2017  | Fugitt et al.      |
| 2003/0085012 A1 | 5/2003  | Jones et al.       |
| 2004/0065423 A1 | 4/2004  | Swerin et al.      |
| 2004/0229063 A1 | 11/2004 | Concannon et al.   |
| 2005/0039872 A1 | 2/2005  | Kimura et al.      |
| 2006/009566 A1  | 1/2006  | Jones et al.       |
| 2006/0124033 A1 | 6/2006  | Pruett et al.      |
| 2007/0169902 A1 | 7/2007  | Brelsford et al.   |
| 2008/0060774 A1 | 3/2008  | Zuraw et al.       |
| 2008/0311416 A1 | 12/2008 | Kelly et al.       |
| 2009/0236062 A1 | 9/2009  | Fugitt             |
| 2015/0136349 A1 | 5/2015  | Pietikainen et al. |

**FOREIGN PATENT DOCUMENTS**

|    |                |         |
|----|----------------|---------|
| EP | 0448332 A1     | 9/1991  |
| EP | 1470289 A1     | 10/2004 |
| JP | 01-118692      | 5/1989  |
| JP | 2009001953 A   | 1/2009  |
| JP | 2009013513 A   | 1/2009  |
| WO | 98/51860 A1    | 11/1998 |
| WO | 01/14014 A1    | 3/2001  |
| WO | 2006/033952 A1 | 3/2006  |
| WO | 2009/091406 A1 | 7/2009  |

**OTHER PUBLICATIONS**

Steffner et al., Influence of the calendering conditions on the structure and the properties of woodfree paper—A comparison between soft nip calendering and hard nip calendering, *Nordic Pulp & Paper Research Journal*, vol. 13, No. 1 (2018).

Rättö, Description and analysis of paper deformation in a calender nip effects of high roll temperatures and thickness variations, *Nordic Pulp & Paper Research Journal*, vol. 17, No. 2 (2002).

Endres et al., Influence of calendering conditions on paper surface characteristics : a comparison between hard-nip, soft-nip, and extended soft-nip calendering, *TAPPI Journal*, vol. 4, No. 9, pp. 9-14 (2005).

**Primary Examiner — Mark Halpern**

(74) **Attorney, Agent, or Firm — Walters & Wasylyna LLC**

(57) **ABSTRACT**

A method for manufacturing a paperboard structure includes passing a paperboard substrate through a hot-hard calender to yield a calendered paperboard substrate, the hot-hard calender including a nip defined by a thermo-roller and a counter roller, wherein a contact surface of the thermo-roller is heated to an elevated temperature. The method then includes applying a basecoat to the calendered paperboard substrate to yield a basecoated paperboard substrate, the basecoat includes a basecoat binder and a basecoat pigment blend. The method further includes applying a topcoat to the basecoated paperboard substrate.



FIG. 1



FIG. 2



FIG. 3



FIG. 4



FIG. 5



FIG. 6



FIG. 7



FIG. 8



FIG. 9



FIG. 10

## 1

**SMOOTH AND LOW DENSITY  
PAPERBOARD STRUCTURES AND  
METHODS FOR MANUFACTURING THE  
SAME**

## PRIORITY

This application is a divisional of U.S. Ser. No. 16/869,156 filed on May 7, 2020, which claims priority from U.S. Ser. No. 62/846,278 filed on May 10, 2019. The entire contents of U.S. Ser. No. 16/869,156 and 62/846,278 are incorporated herein by reference.

## FIELD

The present patent application relates to smooth, low-density paperboard and to methods for manufacturing the same.

## BACKGROUND

Paperboard is used in various packaging applications. For example, aseptic liquid packing paperboard is used for packaging beverage cartons, boxes and the like. Therefore, customers often prefer paperboard having a generally smooth surface with few imperfections to facilitate the printing of high quality text and graphics, thereby increasing the visual appeal of products packaged in paperboard.

Conventionally, paperboard smoothness is achieved by a wet stack calendering process in which the paperboard is rewetted and passed through a calendering device having two or more hard rolls. The wet stack calendering process smooths the paperboard by compressing the fiber network (e.g., applies a nip load) to reduce the pits and crevices in the raw stock board. Therefore, smooth paperboard is typically more dense (e.g., less bulky) than less smooth paperboard.

Nonetheless, low density is a desirable quality in many paperboard applications. However, preparing a smooth paperboard using conventional processes generally requires substantially increasing paperboard density.

Accordingly, those skilled in the art continue with research and development efforts in the field of paperboard manufacturing.

## SUMMARY

In one aspect, the disclosed method for manufacturing a paperboard structure includes passing a paperboard substrate through a hot-hard calender to yield a calendered paperboard substrate, the hot-hard calender including a nip defined by a thermo-roller and a counter roller, wherein a contact surface of the thermo-roller is heated to an elevated temperature. The disclosed method then includes applying a basecoat to the calendered paperboard substrate to yield a basecoated paperboard substrate, the basecoat includes a basecoat binder and a basecoat pigment blend. The disclosed method further includes applying a topcoat to the basecoated paperboard substrate. The paperboard structure has a basis weight, a caliper thickness and a Parker Print Surf smoothness, the Parker Print Surf smoothness being at most about 3 microns, the basis weight being at most  $Y_2$  pounds per 3000 ft<sup>2</sup>, wherein  $Y_2$  is a function of the caliper thickness (X) in point (1 point=one thousandth of an inch) and is calculated as follows:

$$Y_2 = 3.71 + 13.14X - 0.1602X^2$$

## 2

In another aspect, the disclosed method for manufacturing a paperboard structure includes passing a paperboard substrate through a hot-hard calender to yield a calendered paperboard substrate, the hot-hard calender including a nip defined by a thermo-roller and a counter roller, wherein a contact surface of the thermo-roller is heated to an elevated temperature. The disclosed method then includes applying a basecoat to the calendered paperboard substrate to yield a basecoated paperboard substrate, the basecoat includes a basecoat binder and a basecoat pigment blend. The disclosed method further includes applying a topcoat to the basecoated paperboard substrate.

Other aspects of the disclosed method for manufacturing a paperboard structure, and the paperboard structures manufactured by such methods, will become apparent from the following detailed description, the accompanying drawings and the appended claims.

## BRIEF DESCRIPTION OF THE DRAWINGS

FIG. 1 is a cross-sectional view of an example smooth, low density paperboard structure.

FIG. 2 is a schematic illustration of a first example of a method for manufacturing a smooth, low density paperboard structure.

FIG. 3 is a schematic illustration of a second example of a method for manufacturing a smooth, low density paperboard structure.

FIG. 4 is a graphical representation of density versus caliper thickness of various examples of the disclosed smooth, low density paperboard structures, as well as prior art examples.

FIG. 5 is a graphical representation of density versus Parker Print Surf smoothness of various examples of the disclosed smooth, low density paperboard structures having a caliper thickness of about 10 points, as well as prior art examples.

FIG. 6 is a graphical representation of density versus Parker Print Surf smoothness of various examples of the disclosed smooth, low density paperboard structures having a caliper thickness of about 14 points, as well as prior art examples.

FIG. 7 is a graphical representation of basis weight versus caliper thickness of various examples of the disclosed smooth, low density paperboards.

FIG. 8 is a graphical representation of basis weight versus caliper thickness for the disclosed smooth, low density paperboards, as well as prior art examples.

FIG. 9 is a graphical representation of basis weight versus caliper thickness of various examples of the disclosed smooth, low density paperboards.

FIG. 10 is a graphical representation of basis weight versus caliper thickness for the disclosed smooth, low density paperboards, as well as prior art examples.

## DETAILED DESCRIPTION

Referring to FIG. 1, an example paperboard structure 10 that may be manufactured using the method 20 disclosed herein is shown. The paperboard structure 10 may have a caliper thickness T and an upper surface S upon which text or graphics may be printed. The paperboard structure also includes a paperboard substrate 12 and a coating structure 19.

The paperboard substrate 12 may be any paperboard material that is capable of being coated, such as with the disclosed basecoat 14. The paperboard substrate 12 may be

bleached, and may be a single-ply substrate or a multi-ply substrate. However, use of an unbleached paperboard substrate **12** is also contemplated. Those skilled in the art will appreciate that the paperboard substrate **12** will be thicker and more rigid than paper. Generally, a paperboard substrate **12** has an uncoated basis weight of about 85 pounds per 3000 ft<sup>2</sup> or more. In one or more examples, however, the paperboard substrate **12** may have an uncoated basis weight of about 100 pounds per 3000 ft<sup>2</sup> or more. One specific, non-limiting example of an appropriate paperboard substrate **12** is solid bleached sulfate (SBS). In one particular example, the paperboard substrate **12** may include a substantially chemically (rather than mechanically) treated fiber, such as an essentially 100 percent chemically treated fiber. Examples of appropriate chemically treated fiber substrates include solid bleached sulfate paperboard or solid unbleached sulfate paperboard.

Additional components, such as binders, fillers, pigments and the like, may be added to the paperboard substrate **12** without departing from the scope of the present disclosure. Furthermore, the paperboard substrate **12** may be substantially free of plastic pigments for increasing bulk, such as hollow plastic pigments or expandable microspheres, or other chemical bulking agents. Still furthermore, the paperboard substrate **12** may be substantially free of ground wood particles.

The coating structure **19** includes a basecoat **14**, a topcoat **18** and may include any number of intermediate coating layers **16**. The basecoat **14**, topcoat **18**, and optional intermediate coating layers **16** may improve the smoothness of the surface **S** of the paperboard structure **10** without substantially reducing the caliper thickness **T** of the paperboard structure **10**. The basecoat **14** is applied first, directly to the paperboard substrate **12**, and may be followed by various intermediate coating layers **16**. The topcoat **18** is applied last to form the outermost layer (e.g., the basecoat is positioned between the topcoat and the paperboard substrate). Once applied, the coating structure may have a total coat weight equal to the combined weight of the individual layers (e.g., basecoat **14**, topcoat **18** and intermediate coating layers **16**). The total coat weight may be measured after the coating structure has been dried. In one example, the coating structure may have a total coat weight, on a dry basis, ranging from about 8 lbs/3000 ft<sup>2</sup> to about 18 lbs/3000 ft<sup>2</sup>. In another example, the coating structure may have a total coat weight, on a dry basis, ranging from about 12 lbs/3000 ft<sup>2</sup> to about 16 lbs/3000 ft<sup>2</sup>.

The basecoat **14** includes a basecoat binder, a basecoat pigment (or basecoat pigment blend) and, optionally, various other components. In one particular implementation, the basecoat pigment blend includes ground calcium carbonate and hyperplaty clay (e.g., clay having a relatively high aspect ratio or shape factor). For example, the basecoat pigment blend may consist essentially of ground calcium carbonate and hyperplaty clay. The terms "aspect ratio" and "shape factor" refer to the geometry of the individual clay particles, specifically to a comparison of a first dimension of a clay particle (e.g., the diameter or length of the clay particle) to a second dimension of the clay particle (e.g., the thickness or width of the clay particle). The terms "hyperplaty," "high aspect ratio" and "relatively high aspect ratio" refer to aspect ratios generally in excess of 40:1, such as 50:1 or more, particularly 70:1 or more, and preferably 90:1 or more.

In one example, the hyperplaty clay of the basecoat pigment blend may include a platy clay wherein, on average, the clay particles have an aspect ratio of about 40:1 or more. In another example, the hyperplaty clay of the basecoat pigment blend may include a platy clay wherein, on average, the clay particles have an aspect ratio of about 70:1 or more. In yet another example, the hyperplaty clay of the basecoat pigment blend may include a platy clay wherein, on average, the clay particles have an aspect ratio of about 90:1 or more. 10 An example of such a clay is BARRISURFTM, which is available from Imerys Pigments, Inc. of Roswell, Ga.

The ground calcium carbonate of the basecoat pigment blend may range from fine to coarse depending on the particle size of the ground calcium carbonate. Wherein about 15 95 percent of the ground calcium carbonate particles are less than about 2 microns in diameter, the ground calcium carbonate is generally considered to be "fine." Wherein about 60 percent of the ground calcium carbonate particles are less than about 2 microns in diameter, the ground 20 calcium carbonate is generally considered to be "coarse." Further, ground calcium carbonate may also be "extra coarse" when about 35 percent of the ground calcium carbonate particles are less than about 2 microns in diameter.

In one example, the basecoat pigment blend may include 25 ground calcium carbonate wherein about 60 percent of the calcium particles are less than about 2 microns in diameter. An example of such a ground calcium carbonate is HYDROCARB® 60 available from Omya AG of Oftringen, Germany. In another example, the basecoat pigment blend may 30 include ground calcium carbonate wherein about 45 percent of the calcium particles are less than about 2 microns in diameter. In yet another example, the basecoat pigment blend may include ground calcium carbonate wherein about 35 percent of the calcium particles are less than about 2 35 microns in diameter.

The ratio of ground calcium carbonate to hyperplaty clay in the basecoat pigment blend may vary. In one example, the ground calcium carbonate may be at least about 10 percent by weight of the basecoat pigment blend and at most about 40 60 percent by weight of the basecoat pigment blend. In another example, the ground calcium carbonate may be at least about 40 percent by weight of the basecoat pigment blend and at most about 60 percent by weight of the basecoat pigment blend. In yet another example, the basecoat pigment blend includes about 50 percent by weight ground calcium carbonate and about 50 percent by weight hyperplaty clay.

The basecoat binder may be any suitable binder and may be selected based on a variety of manufacturing considerations. In one example, the basecoat binder may include 50 latex. In another example, the basecoat binder may include styrene-acrylic latex. Examples of suitable basecoat binders include RHOPLEX P-308 available from the Dow Chemical Corporation of Midland, Mich. and RESYN 1103 available from Celanese International Corporation of Irving, Tex. 55 Likewise, the various other basecoat components may vary as well depending on manufacturing considerations. In one or more examples, however, the various other basecoat components may include a dispersant. An example of such a dispersant is BERCHEM 4842 available from Bercen, Inc. of Denham Springs, La.

The topcoat **18** may be applied to the paperboard substrate **12** after a basecoat **14** has been applied. The topcoat **18** may be any appropriate topcoat and may include a topcoat binder, a topcoat pigment blend, and various other components. The 60 topcoat pigment blend may include calcium carbonate and clay. In one example, calcium carbonate may be at least about 50 percent by weight of the topcoat pigment blend and

at most about 70 percent by weight of the topcoat pigment blend. In another example, the topcoat pigment blend may include about 60 percent by weight calcium carbonate and about 40 percent by weight clay. The topcoat pigment blend may vary or be substantially similar to the basecoat pigment blend in terms of the coarseness of the calcium carbonate and the aspect ratio of the clay. In one example, the topcoat pigment blend may include fine ground calcium carbonate, such as HYDROCARB® 90 available from Omya AG of Offingen, Germany. In another example, the topcoat pigment blend may include clay, such as Kaofine 90 available from Thiele Kaolin Company of Sandersville, Ga. In yet another example, the topcoat pigment blend may include fine ground calcium carbonate and clay.

The topcoat binder may be any suitable binder and may be selected based on a variety of manufacturing considerations. In one example, the basecoat binder may include latex. In another example, the basecoat binder may include styrene-acrylic latex. Examples of suitable basecoat binders include RHOPLEX P-308 available from the Dow Chemical Corporation of Midland, Mich. and RESYN 1103 available from Celanese International Corporation of Irving, Tex. The various other topcoat components may similarly include any suitable additive such as a dispersant, a lubricant and polyvinyl alcohol. An example of a suitable lubricant is NOP-COTE C-104 available from Geo Specialty Chemicals, Inc. of Lafayette, Ind. An example of a suitable polyvinyl alcohol is SEKISUI SELVOL 205 available from Sekisui Specialty Chemicals America of Dallas, Tex.

Referring to FIG. 2, an example method 20 for manufacturing a paperboard structure 10 is illustrated. The method 20 may begin at the head box 22 which may discharge a fiber slurry onto a Fourdrinier 24 to form a paperboard substrate 26. The paperboard substrate 26 may pass through one or more wet presses 28 and, optionally through one or more dryers 30. A size press 32 may be used and may slightly reduce the caliper thickness of the paperboard substrate 26 and an optional dryer 34 may additionally dry the paperboard substrate 26.

The paperboard substrate 26 then passes through a hot-hard calender 60 to yield a calendered paperboard substrate. The hot-hard calender 60 includes a nip 62 wherein a nip load may be applied to the paperboard substrate 26. Further, the nip 62 is defined by a counter roller 68 and a thermo-roller 64. The counter roller 68 and/or the thermo-roller 64 may be made from a metallic material, such as steel or iron, or other suitably hard materials, such as a heat-resistant resin composite. The thermo-roller 64 includes at least one contact surface 66 (for contacting the paperboard substrate 26) that is heated to an elevated temperature. In another example, shown in FIG. 3, the hot-hard calender 60 may alternatively include a nip 62 and a second nip 63 wherein the nip 62 is defined by a thermo-roller 64 and a counter roller 68, and the second nip 63 is defined by same thermo-roller 64 and a second counter roller 69.

The nip load applied to the paperboard substrate 12 may vary. In an example, the nip load applied to the paperboard substrate 12 may range from about 20 pli (pounds per linear inch) to about 500 pli. In an example, the nip load applied to the paperboard substrate 12 may range from about 20 pli to about 350 pli. In an example, the nip load applied to the paperboard substrate 12 may range from about 20 pli to about 160 pli. In an example, the nip load applied to the paperboard substrate 12 may range from about 30 pli to about 140 pli.

While passing the paperboard substrate 12 through the hot-hard calender 60, the contact surface 66 of the thermo-

roller 64 is heated to an elevated temperature so as to heat the paperboard substrate 12 as it is being calendered. In one example, the elevated temperature may be at least 250° F. In another example, the elevated temperature may be at least 300° F. In another example, the elevated temperature may be at least 400° F. In yet another example, the elevated temperature may be at least 500° F.

After being calendered, the paperboard substrate 12 may pass through another optional dryer 38 and to the first coater 40. The first coater 40 may be a blade coater or the like and may apply the basecoat 14 onto the paperboard substrate 12, thereby yielding a basecoated paperboard substrate. An optional dryer 42 may dry, at least partially, the basecoat 14 prior to application of another coat. A second coater 44 may then apply a topcoat 18 to the basecoated paperboard substrate, thereby yielding the paperboard structure. Another optional dryer 46 may finish the drying process before the paperboard substrate 26 proceeds to the optional gloss calender 48 and the paperboard substrate 26 is rolled onto a reel 50. Those skilled in the art will appreciate that additional coaters may be utilized after the application of the basecoat 14 and before the application of the topcoat 18 without departing from the scope of the present disclosure. These additional coaters may apply, for example, intermediate coating layers 16.

At this point, those skilled in the art will appreciate that the basecoats 14, topcoats 18, intermediate coating layers 16 and associated application techniques disclosed above may substantially increase the smoothness of the resulting paperboard structure 10 while essentially maintain the caliper thickness of the paperboard substrate throughout the coating process, thereby yielding a smooth (e.g., a Parker Print Surf smoothness of 3 microns or less), low density paperboard structure 10.

## EXAMPLES

Specific example of smooth, low density paperboard prepared in accordance with the present disclosure are presented below.

### Example 1

An uncoated solid bleached sulfate (SBS) paperboard substrate having a basis weight of about 145 lbs/3000 ft<sup>2</sup> was prepared using a full-scale production process. Starch was applied to the surface of the SBS board during production.

The paperboard substrate was calendered by Valmet Technologies Oy of Järvenpää, Finland, using a hot-hard calender having a two roll (e.g., one nip) design. The hot-hard calender included one thermo-roller and one counter roller. The nip load was about 140 pli and the surface temperature of the thermo-roller was about 480° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 14 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 164 lbs/3000 ft<sup>2</sup>, a caliper of about 0.0155 inches (15.5 points), and a Parker Print Surf (PPS 10S) roughness of about 1.9 microns.

#### Example 2

An uncoated solid bleached sulfate (SBS) paperboard substrate having a basis weight of about 145 lbs/3000 ft<sup>2</sup> was prepared using a full-scale production process. Starch was applied to the surface of the SBS board during production.

The paperboard substrate was calendered by Valmet Technologies Oy of Järvenpää, Finland using a hot-hard calender having a two roll (e.g., one nip) design. The hot-hard calender included one thermo-roller and one counter roller. The nip load was about 140 pli and the surface temperature of the thermo-roller was about 480° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 12 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 161 lbs/3000 ft<sup>2</sup>, a caliper of about 0.0151 inches (15.1 points), and a Parker Print Surf (PPS 10S) roughness of about 1.9 microns.

#### Example 3

An uncoated solid bleached sulfate (SBS) paperboard substrate having a basis weight of about 145 lbs/3000 ft<sup>2</sup> was prepared using a full-scale production process. Starch was applied to the surface of the SBS board during production.

The paperboard substrate was calendered by Valmet Technologies Oy of Järvenpää, Finland using a hot-hard calender having a two roll (e.g., one nip) design. The hot-hard calender included one thermo-roller and one counter roller. The nip load was about 140 pli and the surface temperature of the thermo-roller was about 480° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-

Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 16 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 164 lbs/3000 ft<sup>2</sup>, a caliper of about 0.0153 inches (15.3 points), and a Parker Print Surf (PPS 10S) roughness of about 1.7 microns.

#### Example 4

An uncoated solid bleached sulfate (SBS) paperboard substrate having a basis weight of about 104 lbs/3000 ft<sup>2</sup> was prepared using a full-scale production process. Starch was applied to the surface of the SBS board during production.

The paperboard substrate was calendered by Valmet Technologies Oy of Järvenpää, Finland using a hot-hard calender having a three roll (e.g., two nip) design. The hot-hard calender included one thermo-roller and one counter roller. The nip load was about 90 pli and the surface temperature of the thermo-roller was about 500° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 12 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 119 lbs/3000 ft<sup>2</sup>, a caliper of about 0.0105 inches (10.5 points), and a Parker Print Surf (PPS 10S) roughness of about 1.3 microns.

#### Example 5

An uncoated solid bleached sulfate (SBS) paperboard substrate having a basis weight of about 104 lbs/3000 ft<sup>2</sup> was prepared using a full-scale production process. Starch was applied to the surface of the SBS board during production.

The paperboard substrate was calendered by Valmet Technologies Oy of Järvenpää, Finland using a hot-hard calender having a three roll (e.g., two nip) design. The hot-hard calender included one thermo-roller and one counter roller. The nip load was about 90 pli and the surface temperature of the thermo-roller was about 500° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 12 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 117 lbs/3000 ft<sup>2</sup>, a caliper of about 0.0103 inches (10.3 points), and a Parker Print Surf (PPS 10S) roughness of about 1.4 microns.

#### Example 6

An uncoated solid bleached sulfate (SBS) paperboard substrate having a basis weight of about 104 lbs/3000 ft<sup>2</sup> was prepared using a full-scale production process. Starch was applied to the surface of the SBS board during production.

The paperboard substrate was calendered by Valmet Technologies Oy of Järvenpää, Finland using a hot-hard calender having a two roll (e.g., one nip) design. The hot-hard calender included one thermo-roller and one counter roller. The nip load was about 90 pli and the surface temperature of the thermo-roller was about 500° F.

A basecoat was prepared as a mixture of 50 parts high aspect ratio clay, 50 parts of extra coarse calcium carbonate, 17 parts of a Styrene-Acrylic Binder, 4 parts of a surfactant stabilized polyvinyl acetate, and minor amounts of dispersant.

A topcoat was also prepared as a mixture of 60 parts of fine carbonate, 40 parts of fine clay, 9 parts of Styrene-Acrylic Binder, 3 parts of a surfactant stabilized polyvinyl acetate, less than 2% of Polyvinyl Alcohol, and minor amounts of dispersant and lubricant.

The calendered paperboard substrate was then coated on one side (C1S) with the basecoat and then the topcoat. The total quantity of applied coating (basecoat and topcoat) was about 15 lbs/3000 ft<sup>2</sup>.

The coated paperboard structure was then final calendered using a gloss-type calender at the WestRock pilot plant. The gloss-type calender included a counter roller covered with a soft polyurethane cover and applied a nip load of around 150 pli while roller surface temperatures were maintained around 200° F.

The coated paperboard structure had a total basis weight of 120 lbs/3000 ft<sup>2</sup>, a caliper of about 0.0106 inches (10.6 points), and a Parker Print Surf (PPS 10S) roughness of about 1.3 microns.

#### Comparative Examples 1-6

For each of the above examples, a Comparative Example was also prepared to demonstrate the improvement presented by the disclosed method (e.g., Comparative Example

1 is comparable to Example 1, Comparative Example 2 is comparable to Example 2, and so on). The paperboard substrate for each Comparative Example was initially prepared in the same manner as the corresponding Example (e.g., uncoated, same basis weight and with starch applied). However, instead of being calendered by a hot-hard calender, the paperboard substrates of the Comparative Examples were calendered using a traditional calender under traditional calendering conditions. Compared to any of the Examples, the nip load applied to the Comparative Examples was much higher at 350 pli and the roller surface temperatures was much lower at 200° F. After being calendered, the Comparative Examples were coated in the same manner and with the same basecoat and topcoat formulations at their corresponding Examples. The Comparative Examples were also final calendered in the same manner as their corresponding Examples.

#### SUMMARY

The results are summarized in Tables 1 and 2 presented below. Table 1 presents the conditions under which the paperboard substrates were calendered prior to being coated and Table 2 presents the resulting data after having been coated.

TABLE 1

|                       | Nip Load<br>(pli) | Roller<br>Surface<br>Temp. (° F.) | Qty of<br>Nips |
|-----------------------|-------------------|-----------------------------------|----------------|
| Example 1             | 140               | 480                               | 1              |
| Example 2             | 140               | 480                               | 1              |
| Example 3             | 140               | 480                               | 1              |
| Example 4             | 90                | 500                               | 2              |
| Example 5             | 90                | 500                               | 2              |
| Example 6             | 90                | 500                               | 1              |
| Comparative Example 1 | 350               | 200                               | 4              |
| Comparative Example 2 | 350               | 200                               | 4              |
| Comparative Example 3 | 350               | 200                               | 4              |
| Comparative Example 4 | 350               | 200                               | 4              |
| Comparative Example 5 | 350               | 200                               | 4              |
| Comparative Example 6 | 350               | 200                               | 4              |

TABLE 2

|                          | Actual<br>Caliper<br>(points) | Basis<br>Weight<br>(lbs/<br>3,000 ft <sup>2</sup> ) | Density<br>(lbs/<br>3,000 ft <sup>2</sup> /<br>points) | PPS<br>(microns) | Total Coat<br>Weight<br>(lbs/<br>3,000 ft <sup>2</sup> ) |
|--------------------------|-------------------------------|-----------------------------------------------------|--------------------------------------------------------|------------------|----------------------------------------------------------|
| Example 1                | 15.5                          | 164                                                 | 10.6                                                   | 1.9              | 14                                                       |
| Example 2                | 15.1                          | 161                                                 | 10.6                                                   | 1.9              | 12                                                       |
| Example 3                | 15.3                          | 164                                                 | 10.8                                                   | 1.7              | 16                                                       |
| Example 4                | 10.5                          | 119                                                 | 11.3                                                   | 1.3              | 12                                                       |
| Example 5                | 10.3                          | 117                                                 | 11.3                                                   | 1.4              | 12                                                       |
| Example 6                | 10.6                          | 120                                                 | 11.3                                                   | 1.3              | 15                                                       |
| Comparative<br>Example 1 | 14.6                          | 162                                                 | 11.1                                                   | 1.9              | 13                                                       |
| Comparative<br>Example 2 | 14.8                          | 164                                                 | 11.1                                                   | 1.6              | 15                                                       |
| Comparative<br>Example 3 | 14.6                          | 164                                                 | 11.1                                                   | 1.8              | 15                                                       |
| Comparative<br>Example 4 | 10.3                          | 120                                                 | 11.7                                                   | 1.4              | 11                                                       |
| Comparative<br>Example 5 | 10.3                          | 123                                                 | 11.9                                                   | 1.2              | 14                                                       |
| Comparative<br>Example 6 | 10.3                          | 121                                                 | 11.8                                                   | 1.3              | 12                                                       |

As shown in Tables 1 and 2, a comparably smooth paperboard structure may be manufactured using the dis-

## 11

closed method (which utilizes the hot-hard calender) despite applying a significantly lower nip load. The nip loads applied in Examples 1-6 ranged from 60% to 74.3% lower than the nip loads applied in their corresponding Comparative Examples. Without being bound by any particular theory, it is believed that calendering paperboard substrates at significantly higher temperatures may compensate for lower nip loads in achieving a desired smoothness.

The density (e.g., basis weight divided by caliper) versus caliper data from Examples 1-6, together with density versus caliper data for prior art paperboard, is plotted in FIG. 4. 10. Those skilled in the art will appreciate that significantly lower densities are achieved when paperboard is prepared in accordance with the present disclosure. Those skilled in the art will also appreciate that density is a function of caliper, so one should compare individual calipers separately when evaluating Parker Print Surf smoothness (PPS).

FIG. 5 illustrates density versus Parker Print Surf smoothness for a 10 point board (Examples 4-6) in accordance with the present disclosure, plotted against density versus Parker Print Surf smoothness of prior art 10 point board. FIG. 6 20 illustrates density versus Parker Print Surf smoothness of 14 point board (Examples 1-3), plotted against density versus Parker Print Surf smoothness of prior art 14 point board. Those skilled in the art will appreciate that the paperboard of the present disclosure presents significantly lower densities relative to the prior art, while maintaining smoothness (e.g., lower Parker Print Surf smoothness values).

The basis weight versus caliper data from Examples 1-6 is plotted in FIG. 7 and the basis weight versus caliper data for prior art paperboard is plotted in FIG. 8. All the data points from Examples 1-6 fall below curve  $Y_2$ , which is a plot of  $Y_2=3.71+13.14X-0.1602X^2$ , while all of the prior art data is found above curve  $Y_2$ . Furthermore, five of the data points from the disclosed Examples fall below curve  $Y_3$ , which is a plot of  $Y_3=3.63+12.85X-0.1566X^2$ .

Similarly, basis weight versus caliper data of paperboard structures prepared in accordance with the present disclosure is plotted in FIG. 9 and the basis weight versus caliper data for prior art paperboard is plotted in FIG. 10. All of the data points from Examples 1-6 fall below curve  $Y_2'$ , which is a plot of  $Y_2'=35.55+8.173X-0.01602X^2$ , while all of the prior art data is found above curve  $Y_2'$ . Furthermore, three data points fall below curve  $Y_3'$ , which is a plot of  $Y_3'=34.83+8.010X-0.01570X^2$ .

While basis weight data is currently presented in FIGS. 7-10 for caliper thickness of 10 and 14, those skilled in the art will appreciate that since the disclosed method and coatings were capable of achieving surprising low densities while simultaneously maintaining smoothness, it is to be expected that similar low densities and smoothness's may be achieved at other caliper thicknesses. In one or more examples, the paperboard structure may have a Parker Print Surf smoothness of at most 2.5 microns. In one or more examples, the paperboard structure may have a Parker Print Surf smoothness of 2.0 microns. In one or more examples, the paperboard structure may have a Parker Print Surf smoothness of 1.5 microns.

Accordingly, the method of the present disclosure provides desired smoothness (e.g., PPS 10S smoothness below 3 microns), while maintaining low board density (e.g., basis weight below the disclosed thresholds as a function of caliper thickness).

Although various aspects of the disclosed method for manufacturing a paperboard structure, and the paperboard structures manufactured by such methods, have been shown and described, modifications may occur to those skilled in

## 12

the art upon reading the specification. The present patent application includes such modifications and is limited only by the scope of the claims.

5. What is claimed is:

1. A method for manufacturing a paperboard structure comprising:

passing a paperboard substrate through a hot-hard calender to yield a calendered paperboard substrate, said hot-hard calender comprising a nip defined by a thermo-roller and a counter roller, wherein a contact surface of said thermo-roller is heated to an elevated temperature, wherein said elevated temperature is at least 250° F.;

applying a basecoat to said calendered paperboard substrate to yield a basecoated paperboard substrate, said basecoat comprising a basecoat binder and a basecoat pigment blend comprising ground calcium carbonate and hyperplaty clay; and

applying a topcoat to said basecoated paperboard substrate.

2. The method of claim 1 further comprising applying starch to said paperboard substrate prior to said passing said paperboard substrate through said hot-hard calender.

3. The method of claim 1 wherein said hot-hard calender further comprises a second nip defined by said thermo-roller and a second counter roller, and wherein said passing said paperboard substrate comprises passing said paperboard substrate through said nip and said second nip.

4. The method of claim 1 wherein at least one of said thermo-roller and said counter roller comprises a metallic material.

5. The method of claim 1 wherein said passing said paperboard substrate through said hot-hard calender comprises applying a nip load to said paperboard substrate ranging from about 20 pli to about 500 pli.

6. The method of claim 1 wherein said elevated temperature is at least 400° F.

7. The method of claim 1 wherein said elevated temperature is at least 300° F.

8. The method of claim 1 wherein said elevated temperature is at least 500° F.

9. The method of claim 1 wherein said basecoat is applied to only one side of said calendered paperboard substrate.

10. The method of claim 1 further comprising applying an intermediate coating layer to said basecoated paperboard substrate prior to said applying said topcoat.

11. The method of claim 1 wherein said basecoat binder comprises latex.

12. The method of claim 1 wherein said hyperplaty clay has an average aspect ratio of at least about 40:1.

13. The method of claim 1 wherein at most about 60 percent of said ground calcium carbonate of said basecoat pigment blend has a particle size smaller than 2 microns.

14. The method of claim 1 wherein said ground calcium carbonate comprises at least about 10 percent by weight of said basecoat pigment blend and at most about 60 percent by weight of said basecoat pigment blend.

15. The method of claim 1 wherein said topcoat comprises a topcoat binder and a topcoat pigment blend.

16. The method of claim 15 wherein said topcoat binder comprises latex.

17. The method of claim 15 wherein said topcoat pigment blend comprises calcium carbonate and clay.

18. The method of claim 1 wherein said applying said basecoat and said applying said topcoat yields a coating structure on said paperboard substrate, said coating structure

13

having a total coat weight, on a dry basis, ranging from about 8 lbs/3000 ft<sup>2</sup> to about 18 lbs/3000 ft<sup>2</sup>.

**19.** The method of claim 1 wherein said paperboard structure has a basis weight, a caliper thickness and a Parker Print Surf (PPS 10S) smoothness, said Parker Print Surf (PPS 10S) smoothness being at most 3 microns, said basis weight being at most Y<sub>2</sub>' pounds per 3000 ft<sup>2</sup>, wherein Y<sub>2</sub>' is a function of said caliper thickness (X) in points and is calculated as follows:

$$Y_2=3.71+13.14X-0.1602X^2.$$

**20.** The method of claim 19 wherein said Parker Print Surf (PPS 10S) smoothness is at most 2.5 microns.

**21.** The method of claim 1 wherein said paperboard structure has a basis weight, a caliper thickness and a Parker Print Surf (PPS 10S) smoothness, said Parker Print Surf (PPS 10S) smoothness being at most 3 microns, said basis weight being at most Y<sub>2</sub>' pounds per 3000 ft<sup>2</sup>, wherein Y<sub>2</sub>' is a function of said caliper thickness (X) in points and is calculated as follows:

$$Y_2'=35.55+8.173X-0.01602X^2.$$

14

**22.** The method of claim 1 wherein said paperboard structure has a basis weight, a caliper thickness and a Parker Print Surf (PPS 10S) smoothness, said Parker Print Surf (PPS 10S) smoothness being at most 3 microns, said basis weight being at most Y<sub>3</sub> pounds per 3000 ft<sup>2</sup>, wherein Y<sub>3</sub> is a function of said caliper thickness (X) in points and is calculated as follows:

$$Y_3=3.63+12.85X-0.1566X^2.$$

**23.** The method of claim 1 wherein said paperboard structure has a basis weight, a caliper thickness and a Parker Print Surf (PPS 10S) smoothness, said Parker Print Surf (PPS 10S) smoothness being at most 3 microns, said basis weight being at most Y<sub>3</sub>' pounds per 3000 ft<sup>2</sup>, wherein Y<sub>3</sub>' is a function of said caliper thickness (X) in points and is calculated as follows:

$$Y_3'=34.83+8.010X-0.01570X^2.$$

**24.** The method of claim 1 further comprising drying said basecoated paperboard substrate.

\* \* \* \* \*